

## UNITED STATES PATENT OFFICE.

HENRY L. PRESTHOLDT, OF MINNEAPOLIS, MINNESOTA.

## PROCESS OF RENDERING GLUE WATERPROOF.

No Drawing.

Application filed April 2, 1927. Serial No. 180,624.

My invention has for its object to improve the waterproof qualities of glue, and more especially of casein glues used to glue up or unite the various veneers of what is known 5 as plywood. The better grades of casein glue hitherto on the market have a fairly high waterproofing quality, but none thereof have met the severe tests required to pass the grade A specification of the United States Government Bureau of Standards. This grade A demands a very high waterproofing quality, such high quality being required for various kinds of work, such as aeroplanes, pontoons, boats, and the woodwork of staterooms of 10 liners or sea-going vessels.

I have discovered a simple process by which I can give to casein glues the additional water-resisting quality required, for example, to meet the grade A above referred to. More 20 definitely stated, I have discovered that formaldehyde will act upon casein glues to produce the said increased water-proofing quality. In carrying out this process, the casein glue, before being subjected to the 25 action of formaldehyde, is used to glue up the various veneers or elements of the plywood and the glue, after it has set, is subjected to the action of formaldehyde. When the freshly glued plywood has been allowed 30 to stand under pressure for a few hours, more or less, depending on the characteristics of the glue used, it is removed from the clamps or press and is then treated with formaldehyde or formaldehyde compound. Under 35 this treatment, the pores of the wood absorb the formaldehyde to such an extent that it penetrates through the veneers to the glue line or joint and, upon contact of the formaldehyde with the casein, there is formed a compound whose nature is such that it is extremely insoluble in water. As an illustration of the extreme insolubility or water-resisting qualities of the glue thus treated, it may be stated that I have soaked plywood, made and treated as above described, in water for a year without appreciably loosening the veneers.

After the plywood has been treated by this improved process, the panels or glued-up parts are advisably allowed to season for a few days in a well-ventilated place where the odor of the formaldehyde will be caused to disappear. The treatment does not stain or in any way harm the veneer of which the

plywood is composed. The formaldehyde 55 may be applied either in the form of a solution or in gaseous form, and it may be of varying strength. On the market, the formaldehyde is usually purchased in a forty percent (40%) solution, but, of course, I will 60 not in any way limit myself to the strength of such solution. The solution may be sprayed on the wood or the wood may be dipped in the solution or the solution may be applied by the use of a sponge. Within reasonable lengths, 65 the stronger the solution, the quicker is the water-proofing action.

Another good method of treatment is to take the plywood from the pressure device and loosely stack it in a closed room or chamber and there subject it to formaldehyde gas. The gas may be generated in the room or enclosure by oxidizing methyl alcohol in a special burner, such as is frequently used for 70 fumigating.

From what has been said, it will be understood that I do not limit myself to the particular way of bringing the formaldehyde into contact with the casein glue, but desire to claim the same broadly. I have also found 75 that formaldehyde will, to some extent, increase the waterproofing quality even in animal glues.

In practice I have obtained the results above outlined by the use of formaldehyde 80 either in the form of gas or liquid solution but it is possible that other coagulants may be found useful for the same purpose. The important feature of this case is in the time and manner in which the formaldehyde or glue coagulant is applied. The formaldehyde in fluid form, that is, in either liquid solution or in gaseous form, is applied through the pores of the outer wooden plies or 85 portions and comes into contact with the glue which has already hardened and permanently united the wood elements. In this process the waterproofing action of the formaldehyde may be applied long after the glue has hardened and long after the wooden article has been manufactured. As is evident, 90 this process could be carried out only in uniting elements such as wood that are porous so that the liquid or gaseous formaldehyde can reach the glue which, in the completed ply wood or article, is then covered by the outer 100 wooden plies or sections.

While this improved process is especially

desirable for ply wood, it is, nevertheless, highly useful in the treatment of any and all kinds of multi-section wooden or similar porous articles where glue has been previously set to connect wood sections.

What I claim is:

1. The process of increasing the water-proof quality of set glue in previously manufactured multi-section porous articles which 10 consists in applying a fluid glue coagulant to the set glue through the pores of the material.

2. The process of increasing the water-proof quality of set glue in previously manufactured multi-section wooden articles which 15 consists in applying fluid formaldehyde to set glue through the pores of the wood.

3. The process of increasing the water-proof quality of set glue in multi-section wooden articles which consists first in applying 20 glue between the wood elements and allowing the glue to set and permanently unite with the contacting wood, and in thereafter subjecting the glue and the united portions of the wood to the action of a fluid glue co-

agulant applied thereto through the pores of 25 the wood.

4. The process of increasing the water-proof quality of set glue in multi-section wooden articles which consists first in applying 30 glue between the wood elements and allowing the glue to set and permanently unite with the contacting wood, and in thereafter subjecting the glue and the united portions of the wood to the action of formaldehyde applied thereto through the pores of the 35 wood.

5. The process of increasing the water-proof quality of set glue in multi-section wooden articles which consists first in applying 40 casein glue to connect the wood elements and allowing the glue to set and permanently unite with the contacting wood, and in thereafter subjecting the set casein glue and the connected portions of the wood to the action of formaldehyde applied thereto through 45 the pores of the wood.

In testimony whereof I affix my signature.  
HENRY L. PRESTHOLDT.